

## UNITED STATES PATENT OFFICE

2,204,651

PROCESS FOR REFINING LEAD WHICH  
CONTAINS BISMUTH

Jesse O. Betterton and Yurii E. Lebedeff,  
Metuchen, N. J., assignors to American Smelt-  
ing and Refining Company, New York, N. Y.,  
a corporation of New Jersey

No Drawing. Application December 24, 1938,  
Serial No. 247,660

## 10 Claims.

(Cl. 75—78)

This invention relates to the art of lead refining and particularly concerns the removal of bismuth from lead.

It was long since suggested that various metal separations might be effected by fusing the particular metal mixture or alloy and introducing alkali, alkaline earth or rare earth metal reagents therein for the purpose of concentrating one or more of the constituents of the original alloy as a dross or crust which floats upon the molten bath and is readily separated therefrom.

However, early attempts to specifically apply the suggestion to the lead refinery for the removal of bismuth failed and the advent of any successful, commercial process had to await later discoveries, many of which the reader will find discussed or referred to in an article by applicants appearing in Transactions of the American Institute of Mining and Metallurgical Engineers, vol. 121, pages 205-225 (1936).

Following the discoveries aforementioned, their principles were soon adapted by various refineries treating thousands of tons annually of lead containing bismuth in the amounts ordinarily encountered which, as is well known, usually range in the neighborhood of a few hundredths to a few tenths per cent. In this connection it is highly significant to note that, insofar as applicants are aware, all of the refineries referred to employ calcium as a reagent in debismuthizing such lead.

The present invention provides a process for the removal of bismuth from lead which renders the use of calcium unnecessary. This new process is based upon the simultaneous action of magnesium and alkali metal which action was the more incapable of being predicted since none of the alkali metals alone produces any elimination of bismuth and magnesium alone only produces a partial elimination of bismuth in alloys containing a high content thereof.

The process for debismuthizing lead without the aid of calcium which forms the subject of the present invention thus consists essentially in adding to lead which contains bismuth and which has been previously molten, magnesium and alkali metal in suitable quantities and then allowing the metal bath to cool to near its temperature of solidification.

There is thus formed a floating crust containing bismuth, magnesium, alkali metal and lead and which is separated from the bath of metal by any known process.

This floating crust will contain, according to the proportions of magnesium and alkali metal used,

the desired part of the bismuth contained, and up to substantially the whole of the bismuth content. After this treatment the lead ordinarily contains an excess of magnesium and alkali metal from which it can be freed by any known treatment, 5 for example, with chlorine.

For putting the process according to the invention into effect, the magnesium and alkali metal, e. g., sodium, may be employed in the state of pure metals or of alloys with lead or with other 10 metals, and by adding successively or simultaneously to the bath of impure metal to be treated.

If desired, the proportion of magnesium or alkali metal utilized may be diminished and this diminution be compensated by an increase of 15 alkali metal or magnesium taking care always to provide a simultaneous or successive addition of alkali metal and magnesium; one may thus in particular confer upon the refining process additional advantages such as, for example, minimum 20 costs of the reagents employed, greater ease in the treatment of drosses, etc.

It may be noted that if the lead from which the bismuth is to be removed contains, besides bismuth, other impurities, these may be partly or 25 wholly contained in the dross with the bismuth. However, as there are at present efficacious means for the separation of these other current impurities from impure lead, it may be more economical to separate from the lead to be treated the greater 30 part of its other impurities before applying the process of the invention for the removal of bismuth.

The invention is illustrated in the following non-limiting examples:

## Example I

A lead containing 0.30% of bismuth is treated in the fused state with an addition of magnesium equal to eight pounds per short ton and an addition of sodium equal to twelve pounds per short ton. After agitation and cooling to the neighborhood of the temperature of solidification, the floating crust is separated. The lead obtained contains only 0.007% of bismuth.

## Example II

A lead containing 0.045% of bismuth is treated as above with an addition of magnesium equal to four pounds per short ton and an addition 50 of lithium equal to four pounds per short ton. After cooling and separation of the floating crust the lead obtained contains only 0.008% of bismuth.

In neither Example I nor in Example II is any 55

calcium used, the sole debismuthizing reagents being sodium and magnesium in the first example and lithium and magnesium in the second example.

5. The results are remarkable in view of the fact that no substantial reduction of bismuth could have been made in the lead of the examples either with alkali metal or with magnesium, alone.

What is claimed is:

10. 1. Process for refining lead which contains bismuth, consisting in adding to the lead in the molten state magnesium and alkali metal, cooling the metallic bath to the neighborhood of its solidification point and then separating therefrom the floating crust in which the bismuth has collected, said process being performed in the absence of calcium.

15. 2. Process for refining lead which contains bismuth without the aid of calcium, consisting in adding simultaneously to the lead in the molten state magnesium and alkali metal, cooling the metallic bath to the neighborhood of its solidification point and then separating therefrom the floating crust in which the bismuth has collected.

20. 3. Process for refining lead which contains bismuth without the aid of calcium, consisting in adding successively in either sequence to the lead in the molten state magnesium and alkali metal, cooling the metallic bath to the neighborhood of its solidification point and then separating therefrom the floating crust in which the bismuth has collected.

25. 4. Process for refining lead which contains bismuth without the aid of calcium, consisting in adding to the lead in the molten state magnesium and alkali metal in the state of alloys with lead, cooling the metallic bath to the neighborhood of its solidification point and then separating therefrom the floating crust in which the bismuth has collected.

30. 5. Process for refining lead which contains bismuth without the aid of calcium, consisting in adding to the lead in the molten state magnesium and alkali metal in the state of alloys with other metals, cooling the metallic bath to the neighborhood of its solidification point and then separating therefrom the floating crust in which the bismuth has collected.

6. Process for refining lead which contains bismuth without the aid of calcium, consisting in adding to the lead in the molten state magnesium and alkali metal, cooling the metallic bath to the neighborhood of its solidification point, and then separating therefrom the floating crust in which the bismuth has collected, the proportions of magnesium and alkali metal being coordinated in the sense that the proportion of one may be varied within certain limits, this variation being compensated by a corresponding variation in the opposite sense in the proportion of the other.

7. Process for refining lead which contains bismuth, consisting in bringing to simultaneous action on the lead in molten state magnesium and alkali metal, cooling the metallic bath to the neighborhood of its solidification point and then separating therefrom the floating crust in which the bismuth has collected, said process being performed in the absence of calcium.

8. Process for debismuthizing lead which comprises mixing magnesium and alkali metal into a molten body of the lead, cooling same to raise a crust having a higher bismuth content than the original lead, and effecting a separation between said crust and the refined lead, said debismuthization being effected without the aid of calcium reagent.

9. Process for refining lead containing bismuth by adding alkali metal and magnesium to the molten lead and thereafter effecting a separation between the alkali metal-magnesium bismuthides and the main mass of the lead so treated, characterized in that the process is performed without the addition of calcium to the lead.

10. Process for refining lead with respect to bismuth as a contaminant which comprises subjecting the lead in molten state to the conjoint action of sodium and magnesium, concentrating the bismuth as a bismuth-lead-sodium-magnesium product at a temperature favoring such concentration, and effecting a separation between said product and the rest of the lead, said process being carried out in the absence of any effective amount of calcium reagent.

JESSE O. BETTERTON.  
YURII E. LEBEDEFF.